



US007111665B2

(12) **United States Patent**  
**Stewart et al.**

(10) **Patent No.:** **US 7,111,665 B2**  
(45) **Date of Patent:** **Sep. 26, 2006**

- (54) **LUBRICANT FOR IMPROVED SURFACE QUALITY OF CAST ALUMINUM AND METHOD**
- (75) Inventors: **Patricia A. Stewart**, Pittsburgh, PA (US); **James R. Anglin**, Export, PA (US); **Ray T. Richter**, Murrysville, PA (US); **Larry F. Wieserman**, Apollo, PA (US); **Brian C. Reynolds**, Davenport, IA (US); **Dean K. Vinnedge**, Bettendorf, IA (US); **Jim M. Hart**, Davenport, IA (US)

(73) Assignee: **Alcon Inc.**, Pittsburgh, PA (US)

(\*) Notice: Subject to any disclaimer, the term of this patent is extended or adjusted under 35 U.S.C. 154(b) by 0 days.

(21) Appl. No.: **11/196,857**

(22) Filed: **Aug. 4, 2005**

(65) **Prior Publication Data**

US 2006/0089268 A1 Apr. 27, 2006

**Related U.S. Application Data**

(63) Continuation-in-part of application No. 10/974,384, filed on Oct. 26, 2004.

(51) **Int. Cl.**

**B22D 11/07** (2006.01)  
**B28B 7/36** (2006.01)

(52) **U.S. Cl.** ..... **164/492**; 164/268; 164/72; 508/154; 106/38.24

(58) **Field of Classification Search** ..... 164/472, 164/268, 122, 72, 138; 508/154, 156; 106/38, 106/24

See application file for complete search history.

(56) **References Cited**

**U.S. PATENT DOCUMENTS**

4,336,147 A \* 6/1982 Stayner ..... 508/156

4,775,418 A \* 10/1988 Laemmle et al. ..... 106/38.24  
6,269,862 B1 \* 8/2001 Richards et al. ..... 164/472  
6,334,978 B1 1/2002 DeYoung et al. ..... 420/529  
6,412,164 B1 7/2002 DeYoung et al. ..... 29/527.5  
6,725,904 B1 \* 4/2004 Desrosiers et al. ..... 164/444

**FOREIGN PATENT DOCUMENTS**

JP 2000015419 \* 1/2000

\* cited by examiner

*Primary Examiner*—Kevin Kerns

*Assistant Examiner*—I.-H. Lin

(74) *Attorney, Agent, or Firm*—Greenberg Traurig LLP; Harry A. Hild, Jr.

(57) **ABSTRACT**

In a lubricant composition suitable for use in the manufacture of aluminum alloys comprising a lubricant base, the improvement wherein the lubricant composition further comprises: an effective amount of water, surfactant, and a high viscosity organic material having a low vapor pressure. It is believed that this mixture provides a method for uniformly distributing the surface oxide at the meniscus for casting applications and increasing meniscus stability. Uniform distribution of the oxide and increased stability at the meniscus reduces vertical fold formation that can lead to cracks in the aluminum ingot. In addition, the mixture promotes uniform heat transfer around the mold. Uniform heat transfer around the mold allows the solidifying aluminum alloy to stay in contact with the mold longer and form stronger ingot shells. A process for continuous or semi-continuous casting of aluminum alloys via the use of this lubricant composition is also disclosed.

**64 Claims, 6 Drawing Sheets**





FIG.1



FIG.4



FIG.2



*FIG.3a*



*FIG.3b*



FIG. 5





FIG. 7



FIG. 8



FIG. 9

## 1

**LUBRICANT FOR IMPROVED SURFACE  
QUALITY OF CAST ALUMINUM AND  
METHOD**

**CROSS-REFERENCE TO RELATED  
APPLICATIONS**

This application is a continuation-in-part of application Ser. No. 10/974,384, filed on Oct. 26, 2004.

**FIELD OF THE INVENTION**

The invention relates to lubricant formulations for use in the casting of aluminum or aluminum alloy ingots or bodies. In particular, the invention relates to using lubricants containing water, surfactants, and a high viscosity organic material to improve the surface quality of cast ingots or bodies, resulting in enhanced product recovery. A method for producing aluminum or aluminum alloy ingots with enhanced surface quality is also disclosed.

**BACKGROUND OF THE INVENTION**

The casting of alloys may be done by any number of methods known to those skilled in the art, such as direct chill casting (DC), electromagnetic casting (EMC), horizontal direct chill casting (HDC), hot top casting, continuous casting, semi-continuous casting, die casting, roll casting, and sand casting.

Each of these casting methods mentioned above has a set of its own inherent problems, but with each technique, surface imperfections can be an issue. In the aluminum alloy casting art, molten metal (or melt for brevity) surface oxidation can produce various surface imperfections in cast ingots such as pits, vertical folds, oxide patches and the like, which can develop into cracks during casting or in later processing. A crack in an ingot or slab propagates during subsequent rolling, for example, leading to expensive remedial rework or scrapping of the cracked material. One mechanical means of removing surface imperfections from an aluminum alloy ingot is scalping. Scalping involves the machining off of a surface layer along the rolling faces of an ingot after it has solidified. However, scalping results in lost metal.

Rectangular ingot yields for high magnesium alloys, such as 7050 and other 7xxx alloys as well as 5182 and 5083 alloys are especially prone to surface defects and cracking caused by initiation at vertical folds on the surface of the ingot. In the past, beryllium has been added, usually at part per million (ppm) levels to some of these alloys to control melt surface defects, and to prevent magnesium loss due to oxidation. In addition, materials, especially those containing fluorine, such as boron trifluoride and ammonium fluoroborate, have been used to promote uniform oxide distribution and therefore reduce surface defects and cracking. However, the use of these additives can be very costly and beryllium itself may fall into disuse due to allegations regarding health, disposal, and environmental issues that it creates. Furthermore, the use of gases can create toxic and corrosive gaseous atmospheres. For these reasons, suitable replacement strategies to control the nature of oxides during casting are needed.

In the casting of aluminum alloys it is also known in the art to use a mold lubricant. Satisfactory ingot surfaces can be obtained using a lubricant that is effective in keeping aluminum from sticking to the mold at high temperatures used in casting aluminum alloys. In early casting practices,

## 2

greases were commonly employed as mold lubricants. However, with the advent of modern casting methods, including continuous or semi-continuous casting, free flowing oils have been used to provide continuous lubrication and have replaced the use of greases as mold lubricants.

Continuous casting refers to the uninterrupted formation of a cast body or ingot. For example, the body or ingot may be cast on or between belts, as in belt casting; between blocks, as in block casting; or in a mold or die that is open at both ends, as in direct chill (DC) casting. Casting may continue indefinitely if the cast body is subsequently cut into desired lengths. Alternately, the pouring operation may be started and stopped when an ingot of desired length is obtained. The latter situation is referred to as semi-continuous casting.

Continuous lubrication is required for fully continuous casting and offers a number of advantages for semi-continuous casting. These advantages include substantial reduction of flame and smoke, substantial reduction of dragging and tearing tendencies near the end of the cast, and allowing casting practices that produce better quality and more uniform surfaces.

Despite the use of continuous lubrication during casting, a limitation of current ingot casting practice exists in the non-uniform growth of oxide at the meniscus of molten metal at the mold interface. Non-uniform oxide growth at the meniscus of the molten metal and mold interface is particularly problematic for alloying elements that rapidly oxidize in air or in air containing moisture. For example, alloys containing lithium and magnesium may oxidize rapidly and in both cases, the vapor pressure of the element is higher than that of aluminum. As a result, magnesium and lithium may diffuse to the surface of the ingot and react with oxygen or moisture in the ambient air.

Distribution of the surface oxide on the ingot head and at the meniscus plays an important role in fold prevention or formation. Data from previous research shows that humid air can produce an oxide/hydroxide film that protects magnesium-containing alloys from runaway or uncontrolled magnesium oxidation at molten metal temperatures. Since the weight gain of the magnesium-containing alloy is significantly reduced in humid air as compared to dry air, the oxide layer is thinner and the oxide distribution is believed to be more uniform. Another mechanism that plays a part in the transformation of molten metal to solid metal is the heat transfer at the mold wall between the molten metal and lubricant coated mold wall.

In addition, controlling the stability of the meniscus during casting also plays an important role in fold prevention and formation. An unstable meniscus is often observed during casting by the change of the meniscus shape running along and around the mold face. It is believed that increasing the viscosity of the casting lubricant will provide less fluidity and thus greater stability of the molten metal meniscus.

There remains a need for an effective alternative to beryllium and fluorine containing materials to prevent surface imperfections, such as vertical folds, pits, oxide patches and the like from forming during aluminum ingot casting, and to control the nature and distribution of oxides, particularly when casting aluminum that is alloyed with elements like magnesium and lithium. Such an invention would be instrumental in preventing cracks, which can form during casting or can develop in later processing. Finally, the invention preferably would have no adverse affect on alloy properties.

The primary object of the present invention is to provide a lubricant composition that allows for uniform distribution of surface oxide at the meniscus formed between the molten aluminum and the mold during the continuous and semi-continuous casting of aluminum alloy ingots.

Another object of the present invention is to provide a lubricant composition that promotes a uniform and controlled rate of heat transfer at the interface formed between the molten aluminum and the mold during the continuous or semi-continuous casting of aluminum alloy ingots.

A still further object of this invention is to provide a casting lubricant that promotes uniform oxide distribution without requiring the use of toxic and corrosive gaseous atmospheres, and thus eliminating associated emissions and equipment corrosion.

Still another object of this invention is to provide a method that promotes uniform oxide distribution on aluminum alloy ingots or castings that does not require beryllium additions to the alloy and fluorine containing atmospheres.

A final object of the invention is to provide a casting lubricant composition that allows for a stable meniscus during the continuous and semi-continuous casting of aluminum alloy ingots.

These and other objects and advantages are met or exceeded by the instant invention, and will become more fully understood and appreciated with reference to the following description.

#### SUMMARY OF THE INVENTION

In the present invention it is believed that when water, surfactant, and low vapor pressure organic materials having high viscosity are added to casting lubricants, the improved lubricant formulation can provide a method for uniformly distributing the surface oxide at the meniscus in addition to creating a more stable meniscus. Having a stable meniscus with a uniform distribution of oxide reduces vertical fold formation that can lead to cracks in the aluminum ingot. In addition, the mixture promotes uniform heat transfer around the mold. Uniform heat transfer around the mold allows the solidifying aluminum alloy to stay in contact with the mold longer and form a thicker and stronger ingot shell. Water has an extremely high heat of vaporization when compared to other liquids that can further pull heat away from the meniscus and be affecting this interaction. Uniform heat transfer will also lead to reduced vertical fold formation and associated cracking.

Water, surfactant, and organic materials having high viscosity are added to existing lubricant bases to prepare the lubricant formulations of this invention. The lubricant formulation is mixed in a high speed mixing operation, such as blending or shearing, or any other mixing operation known by those skilled in the art to provide stable dispersions, stable emulsions, and/or true solutions. At this stage, the formulation is ready to use as a casting lubricant.

In the process of casting aluminum alloy ingots, the lubricant formulation of this invention is supplied to the oil ring of a cooled continuous or semi-continuous casting mold, which subsequently lubricates the inner wall of the continuous casting mold. Molten aluminum alloy is cast into the mold. It is believed that the lubricant allows for uniform distribution of the surface oxide at the meniscus.

#### BRIEF DESCRIPTION OF THE DRAWINGS

FIG. 1 is a flowchart for preparation of the formulation of the lubricant of the instant invention.

FIG. 2 is a schematic characterization of a DC continuous casting mold used in the method of this invention.

FIGS. 3a and 3b show the faces of aluminum alloy ingots cast with the use of a standard lubricant and the lubricant formulation of the present invention.

FIG. 4 is a graph showing the isothermal thermogravimetric analysis of 5083 aluminum alloy in dry and wet air.

FIG. 5 is a graph showing the isothermal thermogravimetric analysis of 7050 aluminum alloy in dry and wet air.

10 FIG. 6 is a flowchart for preparation of the formulation of a lubricant composition having a lubricant base, water, surfactant, and a high viscosity organic material.

FIG. 7 is a graph showing the kinematic viscosity values for water additions to glycerol trioleate.

15 FIG. 8 is a graph showing the percent change in kinematic viscosity values for different amounts of a single molecular weight poly alpha olefin (PAO 25) in glycerol trioleate.

FIG. 9 is a graph showing the percent change in kinematic viscosity values for three different molecular weight poly 20 alpha olefins at 50 vol % and with 0.1 wt % water in glycerol trioleate.

#### DETAILED DESCRIPTION OF PREFERRED EMBODIMENTS

All component percentages herein are by weight percent unless otherwise indicated. Also, when referring to any numerical range of values, such ranges are understood to include each and every number and/or fraction between the 25 stated range minimum and maximum. A range of about 0.05% to about 0.5% by weight of water, for example, would expressly include all intermediate values of about 0.06, 0.07, and 0.08% water, all the way up to and including 0.4 and 0.49% water. The same applies to each other numerical 30 property and/or elemental range set forth herein.

The instant invention provides a casting lubricant formulation and method for using this formulation that substantially reduce vertical fold formation that can lead to cracks in an aluminum ingot. In particular, it is believed that 40 practice of the instant invention allows for uniform distribution of the surface oxide at the meniscus of the molten aluminum alloy. In addition, practice of the instant invention leads to uniform heat transfer around a casting mold.

Referring now to FIG. 1, a flowchart for preparation of the 45 lubricant of this invention is presented. The invention improves on existing lubricants used in the casting of aluminum and aluminum base alloy ingots and forms, and in the general manufacture of aluminum products, using thermomechanical processes such as, but not limited to, casting, extrusion, hot and cold rolling, and forging.

In a preferred embodiment, an existing aluminum alloy 50 casting lubricant, glycerol trioleate, is used as the lubricant base. This is evidenced by box number 1 in the flow chart. Box number 2 in the flowchart evidences the amount of 55 water and surfactant. About 0.05% to about 0.5% by weight of water could be added to the lubricant base, but about 0.1% to about 0.4% by weight of water is preferred. Similarly, less than about 0.25% by weight of surfactant could be added to the lubricant base, but about 0.05% to about 0.2% of 60 surfactant is preferred. The types of lubricant that can be used include for example, but without limitation, glycerol trioleate, ethyl oleate, methyl oleate, butyl ricinoleate, methyl acetyl ricinoleate, butyl oleate, glycerol triacetyl ricinoleate, butyl acetyl ricinoleate, polyalphaolefins, polyisobutylenes, castor oil, peanut oil, corn oil, canola oil, 65 cottonseed oil, olive oil, rapeseed oil, safflower oil, sesame oil, sunflower oil, soybean oil, linseed oil, coconut oil, palm

kernel oil, neat's-foot oil, lard oil, tallow oil, and combinations thereof. Any type of water can be used, but soft water is preferred. For purposes of this invention, soft water is to be defined as water with a low content of polyvalent cations. It will be appreciated by those of ordinary skill in the art that polyvalent cations are ions that have more than one positive charge. Examples of polyvalent cations are calcium ( $Ca^{+2}$ ), magnesium ( $Mg^{+2}$ ), iron ( $Fe^{+2}$  and  $Fe^{+3}$ ), and aluminum ( $Al^{+3}$ ). The surfactant can be cationic, anionic, nonionic, or combinations thereof. The surfactant used in this invention was Kimberly Clark® Professional Pink Lotion Soap. This soap is available from the Kimberly Clark Corporation. The mixture is then subjected to high shear for about 5 minutes as represented by box number 3 in the flowchart. High shear is defined as at least 100 revolutions per minute (RPM). Shearing devices including, but not limited to, household blenders, can be used to shear the mixture. The lubricant so formulated, as represented by box number 4 in the flowchart, is applied to a casting mold in any manner that is familiar to those skilled in the art of casting aluminum alloys.

It is believed that a major benefit of the lubricant of this invention is realized in uniformly distributing surface oxides at the meniscus during DC casting of aluminum. However, it is recognized by those skilled in the art that the lubricant of this invention can be used in any thermomechanical processing of aluminum and its alloys. These processing steps include, but are not limited to casting, hot and cold rolling, forging, and extrusion.

Referring now to FIG. 2, a cross-section of a DC casting mold 10, which can be used to cast aluminum alloy ingots according to the instant invention, is schematically depicted. The DC casting mold 10 comprises molten metal 11 from a furnace. The molten metal is held in a trough 12. A control pin 13 activates and deactivates the flow of molten metal 11 into a distributor bag 14, which distributes the molten metal into the cooled mold 15. The molten metal 11 in the cooled mold 15 may form an oxide skim 16. The inner wall 17 of the cooled mold 15 is cooled by a liquid cooling jacket 18 that cools the mold 15 and floods the solidified ingot surface 19 with cooling liquid 20. The liquid is preferably water, but could be any liquid suitable for cooling the ingot 22. The liquid flows from a liquid pump (not shown) that is connected to the sides of the cooling jacket 18. The inner wall 17 is also continuously lubricated with a formulation of the instant invention by using an oil ring 21 positioned at or near the meniscus of where the molten metal 11 in the mold 15 contacts the inner wall 17 of the cooled mold 15. An oil ring is preferred, but other methods of continuously lubricating the mold inner wall could be used. In a preferred embodiment, the lubricant formulation comprises about 0.1% to about 0.4% by weight of water and about 0.05% to about 0.2% by weight of surfactant with the remaining percentage being glycerol trioleate base. Molten metal 11 in the mold 15 solidifies into a solidified ingot 22. The solidified ingot 22 rests on a starting block 23. The starting block 23 rests on a starting block holder 24. The starting block holder 24 is attached to a platen 25. The platen can be lowered or raised by a cylinder ram 26. As molten metal 11 in the mold 15 solidifies into a solidified ingot 22, the cylinder ram 26 is lowered, which causes the solidified ingot 22 to also be lowered according to the directional arrows 27 superimposed onto the schematic cross section of the DC mold 10. As the cylinder ram 26 and solidified ingot 22 are lowered, the control pin 13 is activated to allow more molten metal 11 in the trough 12 to flow into the cooled mold 15 via the distributor bag 14, and ingots of aluminum alloy are cast, the length of such ingots being constrained only by the move-

ment of the cylinder ram 26. During the ingot casting operation, the solidified ingot 22 is in contact with the inner wall 17 and is continuously lubricated with the lubricant of this invention via the oil ring 21 or any other method used to continuously lubricate the mold inner wall, thusly providing a process for minimizing undesirable surface defects, such as vertical folds that were described earlier. During the practice of this invention, there is no requirement for the undesirable practice of alloying the aluminum with beryllium, nor is there any reliance on using toxic materials such as ammonium fluoroborate or boron trifluoride to prevent oxidation during casting.

To test the lubricant formulation, a lubricant was formulated according to the teachings of this invention as described in the following example.

#### EXAMPLE I

7200 grams of glycerol trioleate, 8 grams of water, and 4 grams of Kimberly Clark® Professional Pink Lotion Soap were combined and sheared, via use of a household blender, at high speed (1000 RPM) for five minutes. The lubricant formulation was used in the casting of Aluminum Alloy 5083 and 7050. Casting position 1, which was used as the control, utilized only glycerol trioleate as the lubricant. As can be seen in FIG. 3a, the resultant aluminum alloy ingot was covered with vertical folds. Casting position 2 alternated between using glycerol trioleate and the lubricant formulation of the present invention. As represented in FIG. 3b, the resultant aluminum alloy ingot had only a few light vertical folds when the lubricant formulation of the present invention was used.

The distribution of the surface oxide on the ingot head and at the meniscus plays an important role in fold prevention or formation. FIGS. 4 and 5 represent the isothermal thermogravimetric analysis of 5083 and 7050 alloys in dry air 100 and wet air 200, respectively. For purposes of this invention, dry air is air with a dew point of 59° F. or less and wet air with a dew point between 60° F. and 100° F. Data from previous research shows that wet air 200 can produce an oxide/hydroxide film that protects the high magnesium alloy from runaway or uncontrolled magnesium oxidation at molten metal temperatures. Since the weight gain of the magnesium-containing alloys is significantly reduced as compared to dry air 100, the surface oxide is thinner and is believed to be more uniformly distributed. This change in oxide distribution would play a significant role in vertical fold suppression. Introducing the oxygen, in this case in the form of water mixed with oil and surfactant, provides the method for changing the metal oxide distribution at the meniscus. The critical technical part is to form a homogeneous distribution of water in the oil so water would be limited, but available uniformly over the surface of the casting mold and at the meniscus immediately before solidification. The water may be uniformly dispersed in the oil as a stable dispersion, stable emulsion, a true solution, or a combination thereof. For purposes of this application, the term dispersion is defined as the distribution of a substance, as droplets or fine particles, evenly throughout a medium, the term emulsion is defined as distributing a substance throughout a medium via use of an emulsifier, such as a surfactant, to help link the substance and the medium together, and the term true solution is defined as a homogeneous mixture formed by mixing a solid, liquid, or gaseous substance with a liquid or sometimes a gas or solid. Uniformly distributing the water in this manner reduces vertical folds and the possibility of associated cracking by

also controlling the heat transfer between the molten metal and the lubricant interface on the inner wall of the mold, thereby allowing the solidified shell to stay in contact with the mold longer and form a thicker and stronger shell.

In addition to uniform distribution of the surface oxide on the ingot head and at the meniscus and uniform heat transfer around a casting mold, controlling the stability of the meniscus during casting also plays an important role in fold prevention and formation. An unstable meniscus is often observed during casting by the change of the meniscus shape running along and around the mold face. It is believed that increasing the viscosity of the casting lubricant will provide less fluidity and thus greater stability of the molten metal meniscus. A casting lubricant composition that allows for a stable meniscus during the continuous and semi-continuous casting of aluminum alloy ingots is needed. For the purposes of this invention, a stable meniscus can be defined as maintaining a near constant contact angle between the casting mold and the molten aluminum alloy. There is increased resistance to meniscus deformation in order to maintain a constant distance between the molten aluminum and the cold mold surface. It is believed that having a meniscus with increased stability will substantially reduce the possibility of the molten metal from adhering to and being dragged down the side of the mold. Reducing this possibility, in turn, will increase the surface quality of the resultant aluminum alloy ingot or billet.

It is believed that when water, surfactant, and organic materials having high viscosity are added to casting lubricants, the improved lubricant formulation can provide a method for uniformly distributing the surface oxide at the meniscus in addition to creating a more stable meniscus. The organic material would also preferably have a low vapor pressure. A low vapor pressure organic material would be one that has a boiling point above 100° C. Having a stable meniscus with a uniform distribution of oxide reduces vertical fold formation that can lead to cracks in the aluminum ingot or billet. The lubricant formulation is mixed in a high speed mixing operation, such as blending or shearing, or any other mixing operation known by those skilled in the art to provide stable dispersions, stable emulsions, and/or true solutions. At this stage, the formulation is ready to use as a casting lubricant.

In the process of casting aluminum alloy ingots, the lubricant formulation is supplied to the oil ring of a cooled continuous or semi-continuous casting mold, which subsequently lubricates the inner wall of the continuous casting mold. Molten aluminum alloy is cast into the mold. It is believed that the lubricant allows for uniform distribution of the surface oxide at the meniscus in addition to increasing its stability.

Referring to FIG. 6, a flowchart for preparation of the lubricant is presented. The invention improves on existing lubricants used in the casting of aluminum and aluminum base alloy ingots and forms, and in the general manufacture of aluminum products, using thermomechanical processes such as, but not limited to, casting, extrusion, hot and cold rolling, and forging.

In the preferred embodiment, an existing aluminum alloy casting lubricant, glycerol trioleate, is used as the lubricant base. This is evidenced by box number 1 in the flow chart. Box number 2 in the flowchart evidences the amount of water, surfactant, and high viscosity organic material that are mixed with the lubricant base.

About 0.05% to about 0.5% by weight of water could be added to the lubricant base, but about 0.1% to about 0.4% by weight of water is preferred. Similarly, less than about

0.25% by weight of surfactant could be added to the lubricant base, but about 0.05% to about 0.2% of surfactant is preferred. Finally, between about 5% to about 90% by weight of high viscosity organic material could be added to the lubricant base, but between about 10% to about 80% by weight of high viscosity organic material is preferred. The types of lubricant that can be used include for example, but without limitation, glycerol trioleate, ethyl oleate, methyl oleate, butyl ricinoleate, methyl acetyl ricinoleate, butyl oleate, glycerol triacetyl ricinoleate, butyl acetyl ricinoleate, polyalphaolefins, polyisobutylenes, castor oil, peanut oil, corn oil, canola oil, cottonseed oil, olive oil, rapeseed oil, safflower oil, sesame oil, sunflower oil, soybean oil, linseed oil, coconut oil, palm kernel oil, neat's-foot oil, lard oil, tallow oil, and combinations thereof. Any type of water can be used, but soft water is preferred. For the purposes of this invention, soft water is to be defined as water with a low content of polyvalent cations. It will be appreciated by those of ordinary skill in the art that polyvalent cations are ions that have more than one positive charge. Examples of polyvalent cations are calcium ( $Ca^{+2}$ ), magnesium ( $Mg^{+2}$ ), iron ( $Fe^{+2}$  and  $Fe^{+3}$ ), and aluminum ( $Al^{+3}$ ). The surfactant can be cationic, anionic, nonionic, or combinations thereof. The surfactant used in this invention was Kimberly Clark® Professional Pink Lotion Soap. This soap is available from the Kimberly Clark Corporation. A high viscosity organic material is defined as an organic material with a viscosity value of at least 10 centistokes at 100° C. The range of viscosity values for this preferred embodiment is between about 10 centistokes to about 8000 centistokes with a preferred range of about 15 centistokes to about 4000 centistokes at 100° C. The types of high viscosity organic materials that could be used include, for example, but without limitation, poly alpha olefins, polybutylene, castor oil, high molecular weight esters (Oleon radialube 7396, Radialube 7597, and Clariant L-4, all at 40° C.), polyacrylates, Ketjenlube, polyglycerol esters, polyalkylene glycols, polypropylene glycols, polyvinyl alcohols, oligomerized vegetable oils, and stannous octoate.

The mixture is then subjected to high shear for about 5 minutes as represented by box number 3 in the flowchart. High shear is defined as at least 100 revolutions per minute (RPM). Shearing devices including, but not limited to, household blenders, can be used to shear the mixture. The lubricant so formulated, as represented by box number 4 in the flowchart, is applied to a casting mold in any manner that is familiar to those skilled in the art of casting aluminum alloys.

To examine the effect that the high viscosity organic material had on the lubricant base, several tests were performed. Water was mixed with glycerol trioleate at 0.1 and 0.2 wt % under high shear. Depending on the permeability of the lubricant base to water, surfactant could be used. However, for the purposes of these tests, a surfactant was not used. After mixing, the kinematic viscosities were measured at 40° and 100° Celsius to obtain a viscosity index. For the purposes of this invention, kinematic viscosity is defined as a measure of the internal resistance to flow of a liquid under gravity. The kinematic viscosities were about 42 centistokes at 40° C. and about 8 centistokes at 100° C. for 0 wt %, 0.1 wt %, and 0.2 wt % water. As shown in FIG. 7, the values for the kinematic viscosities did not change from that obtained for glycerol trioleate alone. Further tests were made using various amounts of single molecular weight poly alpha olefin having 25 centistokes viscosity at 100° Celsius (PAO 25). PAO 25 was the sole additive to the lubricant base, which was glycerol trioleate. As shown in FIG. 8, at the 50

vol % formulation using PAO 25, the viscosity increased from values obtained for glycerol trioleate by 55% and 32% for measurements made at 40° and 100° Celsius. While the poly alpha olefin 25 provided increased viscosities, higher molecular weight poly alpha olefin materials were evaluated to obtain even greater increases in viscosity values. As shown in FIG. 9, using poly alpha olefin having 40 centistokes at 100° C. (PAO 40) and poly alpha olefin having 100 centistokes at 100° Celsius (PAO 100), both at 50 vol %, the viscosity values increased by 1.5 and 3.5 times that obtained from glycerol trioleate alone. The addition of 0.1 wt % water did not affect the viscosity values for the new formulations shown in FIG. 9. The use of high viscosity organic materials with a lubricant base, such as glycerol trioleate, provides a substantial increase in the viscosity of the lubricant. It is believed that the use of this higher viscosity lubricant during casting of aluminum alloy ingots or billets will provide less fluidity and thus greater stability of the meniscus at the interface between the molten aluminum and the casting mold. Less fluidity and greater stability of the meniscus would improve ingot and billet surface quality, thus enhancing product recovery.

It will be readily appreciated by those skilled in the art that modifications may be made to the invention without departing from the concepts disclosed in the forgoing description. Such modifications are to be considered as included within the following claims unless the claims, by their language, expressly state otherwise. Accordingly, the particular embodiments described in detail herein are illustrative only and are not limiting to the scope of the invention which is to be given the full breadth of the appended claims and any and all equivalents thereof.

What is claimed is:

1. An ingot lubricant composition suitable for use in the manufacture of aluminum alloys comprising: a casting lubricant base selected from the group consisting of solid lubricants, liquid lubricants, grease lubricants, emulsion lubricants, and dispersion lubricants; a homogenous distribution of water in the casting lubricant base, the water ranging about 0.05% to about 0.5% by weight; surfactant, and a high viscosity organic material, wherein the homogenous distribution of water in the casting lubricant base, the surfactant, and the high viscosity organic material provide an ingot lubricant that forms a uniform distribution of surface oxide at a meniscus formed between molten aluminum and an ingot mold sidewall during continuous or semi-continuous casting.

2. The lubricant composition of claim 1 comprising about 0.1% to about 0.4% by weight of said water.

3. The lubricant composition of claim 1 comprising less than about 0.25% by weight of said surfactant.

4. The lubricant composition of claim 3 comprising about 0.05% to about 0.2% by weight of said surfactant.

5. The lubricant composition of claim 1 comprising about 5% to about 90% by weight of high viscosity organic material.

6. The lubricant composition of claim 5 comprising about 10% to about 80% by weight of high viscosity organic material.

7. The lubricant composition of claim 1 wherein said surfactant is selected from the group consisting of: a cationic surfactant, anionic surfactant, nonionic surfactant, or any combination thereof.

8. The lubricant composition of claim 1 wherein said high viscosity organic material is selected from the group consisting of: poly alpha olefins, polybutylene, castor oil, high molecular weight esters, polyacrylates, polyglycerol esters,

polyalkylene glycols, polypropylene glycols, polyvinyl alcohols, oligomerized vegetable oils, and stannous octoate.

9. The lubricant composition of claim 1 wherein the viscosity of said high viscosity organic material comprises between about 10 centistokes to about 8000 centistokes at 100° C.

10. The lubricant composition of claim 9 wherein the viscosity of said high viscosity organic material comprises between about 15 centistokes to about 4000 centistokes at 100° C.

11. The lubricant composition of claim 1 sheared at high speed prior to use in the manufacture of aluminum alloys.

12. A lubricant composition for use in the casting of aluminum alloys comprising:

a casting lubricant base selected from the group consisting of glycerol trioleate, ethyl oleate, methyl oleate, butyl ricinoleate, methyl acetyl ricinoleate, butyl oleate, glycerol triacetyl ricinoleate, butyl acetyl ricinoleate, polyalphaolefins, polyisobutylenes, castor oil, peanut oil, corn oil, canola oil, cottonseed oil, olive oil, rapeseed oil, safflower oil, sesame oil, sunflower oil, soybean oil, linseed oil, coconut oil, palm kernel oil, neat's-foot oil, lard oil, tallow oil, and combinations thereof, a homogenous distribution of water in the casting lubricant base, the water ranging about 0.05% to about 0.5% by weight, surfactant, and high viscosity organic material, wherein the homogenous distribution of water in the casting lubricant base and the surfactant provide an ingot lubricant that forms a uniform distribution of surface oxide at a meniscus formed between molten aluminum and an ingot mold sidewall during continuous or semi-continuous casting.

13. The lubricant composition of claim 12 comprising about 0.1% to about 0.4% by weight of said water.

14. The lubricant composition of claim 12 comprising less than about 0.25% by weight of said surfactant.

15. The lubricant composition of claim 14 comprising about 0.05% to about 0.20% by weight of said surfactant.

16. The lubricant composition of claim 12 comprising about 5% to about 90% by weight of high viscosity organic material.

17. The lubricant composition of claim 16 comprising 10% to about 80% by weight of high viscosity organic material.

18. The lubricant composition of claim 12 wherein said surfactant is selected from the group consisting of: a cationic surfactant, anionic surfactant, nonionic surfactant, or any combination thereof.

19. The lubricant composition of claim 12 wherein said high viscosity organic material is selected from the group consisting of: poly alpha olefins, polybutylene, castor oil, high molecular weight esters, polyacrylates, polyglycerol esters, polyalkylene glycols, polypropylene glycols, polyvinyl alcohols, oligomerized vegetable oils, and stannous octoate.

20. The lubricant composition of claim 12 wherein the viscosity of said high viscosity organic material comprises between about 10 centistokes to about 8000 centistokes at 100° C.

21. The lubricant composition of claim 20 wherein the viscosity of said high viscosity organic material comprises between about 15 centistokes to about 4000 centistokes at 100° C.

22. The lubricant composition of claim 12 sheared at high speed prior to use in the casting of aluminum alloys.

23. A lubricant composition for use in the casting of aluminum alloys comprising:

## 11

a casting lubricant oil base selected from the group consisting of glycerol trioleate, ethyl oleate, methyl oleate, butyl ricinoleate, methyl acetyl ricinoleate, butyl oleate, glycerol triacetyl ricinoleate, butyl acetyl ricinoleate, castor oil, peanut oil, corn oil, canola oil, cottonseed oil, olive oil, rapeseed oil, safflower oil, sesame oil, sunflower oil, soybean oil, linseed oil, coconut oil, palm kernel oil, neat's-foot oil, lard oil, tallow oil, and combinations thereof; a homogenous distribution of water in the casting lubricant base, the water ranging about 0.05% to about 0.5% by weight; surfactant, and high viscosity organic material, wherein the homogenous distribution of water in the casting lubricant base, the surfactant, and the high viscosity organic material provide an ingot lubricant that forms a uniform distribution of surface oxide at a meniscus formed between molten aluminum and an ingot mold sidewall during continuous or semi-continuous casting.

24. The lubricant composition of claim 23 comprising about 0.1% to about 0.4% by weight of said water.

25. The lubricant composition of claim 23 comprising less than about 0.25% by weight of said surfactant.

26. The lubricant composition of claim 25 comprising about 0.05% to about 0.20% by weight of said surfactant.

27. The lubricant composition of claim 23 comprising about 5% to about 90% by weight of high viscosity organic material.

28. The lubricant composition of claim 27 comprising 10% to about 80% by weight of high viscosity organic material.

29. The lubricant composition of claim 23 wherein said surfactant is selected from the group consisting of: a cationic surfactant, anionic surfactant, nonionic surfactant, or any combination thereof.

30. The lubricant composition of claim 23 wherein said high viscosity organic material is selected from the group consisting of: poly alpha olefins, polybutylene, castor oil, high molecular weight esters, polyacrylates, polyglycerol esters, polyalkylene glycols, polypropylene glycols, polyvinyl alcohols, oligomerized vegetable oils, and stannous octoate.

31. The lubricant composition of claim 23 wherein the viscosity of said high viscosity organic material comprises between about 10 centistokes to about 8000 centistokes at 100° C.

32. The lubricant composition of claim 31 wherein the viscosity of said high viscosity organic material comprises between about 15 centistokes to about 4000 centistokes at 100° C.

33. The lubricant of claim 23 sheared at high speed prior to use in the casting of aluminum alloys.

34. A lubricant composition for use in the casting of aluminum alloys comprising: an existing casting lubricant oil base selected from the group consisting of glycerol trioleate, castor oil, and combinations thereof, a homogenous distribution of water in the casting lubricant base, the water ranging about 0.05% to about 0.5% by weight; surfactant, and high viscosity organic material, wherein the homogenous distribution of water in the casting lubricant base, the surfactant and the high viscosity organic material provide an ingot lubricant that forms a uniform distribution of surface oxide at a meniscus formed between molten aluminum and an ingot mold sidewall during continuous or semi-continuous casting.

35. The lubricant composition of claim 34 comprising about 0.10% to about 0.40% by weight of said water.

## 12

36. The lubricant composition of claim 34 comprising less than about 0.25% by weight of said surfactant.

37. The lubricant composition of claim 36 comprising about 0.05% to about 0.20% by weight of said surfactant.

38. The lubricant composition of claim 34 comprising about 5% to about 90% by weight of high viscosity organic material.

39. The lubricant composition of claim 38 comprising 10% to about 80% by weight of high viscosity organic material.

40. The lubricant composition of claim 34 wherein said surfactant is selected from the group consisting of: a cationic surfactant, anionic surfactant, nonionic surfactant, or any combination thereof.

41. The lubricant composition of claim 34 wherein said high viscosity organic material is selected from the group consisting of: poly alpha olefins, polybutylene, castor oil, high molecular weight esters, polyacrylates, polyglycerol esters, polyalkylene glycols, polypropylene glycols, polyvinyl alcohols, oligomerized vegetable oils, and stannous octoate.

42. The lubricant composition of claim 34 wherein the viscosity of said high viscosity organic material comprises between about 10 centistokes to about 8000 centistokes at 100° C.

43. The lubricant composition of claim 42 wherein the viscosity of said high viscosity organic material comprises between about 15 centistokes to about 4000 centistokes at 100° C.

44. The lubricant of claim 34 sheared at high speed prior to use in the casting of aluminum alloys.

45. An ingot lubricant composition for use in the casting of aluminum alloys comprising glycerol trioleate, about 0.05% to about 0.50% by weight of water, less than about 0.25% by weight of surfactant, and about 5% to about 90% by weight of high viscosity organic material.

46. The lubricant composition of claim 45 comprising about 0.1% to about 0.4% by weight of said water.

47. The lubricant composition of claim 45 comprising about 0.05% to about 0.2% by weight of said surfactant.

48. The lubricant composition of claim 45 comprising about 10% to about 80% by weight of high viscosity organic material.

49. The lubricant composition of claim 45 wherein said surfactant is selected from the group consisting of: a cationic surfactant, anionic surfactant, nonionic surfactant, or any combination thereof.

50. The lubricant composition of claim 45 wherein said high viscosity organic material is selected from the group consisting of: poly alpha olefins, polybutylene, castor oil, high molecular weight esters, polyacrylates, polyglycerol esters, polyalkylene glycols, polypropylene glycols, polyvinyl alcohols, oligomerized vegetable oils, and stannous octoate.

51. The lubricant composition of claim 45 wherein the viscosity of said high viscosity organic material comprises between about 10 centistokes to about 8000 centistokes at 100° C.

52. The lubricant composition of claim 51 wherein the viscosity of said high viscosity organic material comprises between about 15 centistokes to about 4000 centistokes at 100° C.

53. The lubricant of claim 45 sheared at high speed prior to use in the casting of aluminum alloys.

54. A process for the continuous or semi-continuous casting of aluminum alloys wherein molten aluminum alloy

## 13

is cast into a cooled mold having a lubricated inner mold wall, said process comprising the steps of:

- a) lubricating the inner wall of a cooled, continuous or semi-continuous casting mold with a lubricant composition comprising:
  - i) a casting lubricant base selected from the group consisting of glycerol trioleate, ethyl oleate, methyl oleate, butyl ricinoleate, methyl acetyl ricinoleate, butyl oleate, glycerol triacetyl ricinoleate, butyl acetyl ricinoleate, polyalphaolefins, polyisobutylenes, castor oil, peanut oil, corn oil, canola oil, cottonseed oil, olive oil, rapeseed oil, safflower oil, sesame oil, sunflower oil, soybean oil, linseed oil, coconut oil, palm kernel oil, neat's-foot oil, lard oil, tallow oil, and combinations thereof,
  - a homogenous distribution of water in the casting lubricant base, the water ranging about 0.05% to about 0.5% by weight; surfactant, and high viscosity organic material; and
  - b) casting a molten aluminum alloy into said mold, wherein said lubricant is in continuous contact with a meniscus formed between the molten aluminum alloy and the mold, wherein the homogeneous distribution of water in the casting lubricant base allows for uniform distribution of the surface oxide and increased stability at the meniscus of said lubricated inner mold wall and said molten aluminum base alloy.
55. The process of claim 54 comprising about 0.10% to about 0.40% by weight of said water.

## 14

- 56. The process of claim 54 comprising less than about 0.25% by weight of said surfactant.
- 57. The process of claim 56 comprising about 0.05% to about 0.20% by weight of said surfactant.
- 58. The process of claim 54 comprising about 5% to about 90% by weight of high viscosity organic material.
- 59. The process of claim 58 comprising 10% to about 80% by weight of high viscosity organic material.
- 10 60. The process of claim 54 wherein said surfactant is selected from the group consisting of: a cationic surfactant, anionic surfactant, nonionic surfactant, or any combination thereof.
- 15 61. The process of claim 54 wherein said high viscosity organic material is selected from the group consisting of: poly alpha olefins, polybutylene, castor oil, high molecular weight esters, polyacrylates, polyglycerol esters, polyalkylene glycols, polypropylene glycols, polyvinyl alcohols, oligomerized vegetable oils, and stannous octoate.
- 20 62. The process of claim 54 wherein the viscosity of said high viscosity organic material comprises between about 10 centistokes to about 8000 centistokes at 100° C.
- 25 63. The process of claim 62 wherein the viscosity of said high viscosity organic material comprises between about 15 centistokes to about 4000 centistokes at 100° C.
- 64. The process of claim 54 sheared at high speed prior to use in the casting of aluminum alloys.

\* \* \* \* \*

UNITED STATES PATENT AND TRADEMARK OFFICE  
**CERTIFICATE OF CORRECTION**

PATENT NO. : 7,111,665 B2  
APPLICATION NO. : 11/196857  
DATED : September 26, 2006  
INVENTOR(S) : Patricia A. Stewart et al.

Page 1 of 1

It is certified that error appears in the above-identified patent and that said Letters Patent is hereby corrected as shown below:

On the Title Page, Section (73) Assignee: delete "Alcon" and insert --Alcoa--.

On the Title Page, Section (75) Inventors: On the seventh inventor, delete the middle initial "M." and insert --N--.

Signed and Sealed this

First Day of April, 2008



JON W. DUDAS  
*Director of the United States Patent and Trademark Office*